

Patented Oct. 22, 1929

1,732,915

# UNITED STATES PATENT OFFICE

BYRAMJI D. SAKLATWALLA, OF CRAFTON, PENNSYLVANIA, ASSIGNOR TO VANADIUM CORPORATION OF AMERICA, OF BRIDGEVILLE, PENNSYLVANIA, A CORPORATION OF DELAWARE

ALLOY OF ALUMINUM, SILICON, AND IRON

No Drawing.

Application filed February 2, 1928. Serial No. 251,466.

This invention relates to an alloy containing aluminum, silicon, and iron, and especially to an alloy suitable for addition to molten steel for the purpose of obtaining sound, 5 dense ingots when such steel solidifies.

The use of metallic aluminum for the purpose of scavenging molten steel is very well known and is more or less universally used in steel manufacturing practice. Its use, however, is combined with very marked deficiencies so that, while the aluminum frees the molten steel of impurities, such as iron oxide, by chemically reacting with it, the product formed from such reaction, namely, 10 alumina, remains entrapped in the steel, thus imparting to it several objectionable qualities. Moreover, the amount of alumina remaining entrapped in the steel is not always the same and consequently ingots are obtained which 15 have varying physical qualities, such as ductility, although of the same chemical composition. The presence of alumina in aluminum treated steel can be always detected by means of the microscope and it is well recognized that the aluminum content found in such steel is not in the form of metallic aluminum but chemically combined with oxygen as alumina. If any metallic aluminum were residually present, it would be very 20 helpful in densifying the steel and its presence would be a full assurance of the perfect scavenging action of the balance of the aluminum added. Metallic aluminum for the purpose of addition to steel further has the disadvantage of entering into reaction at high 25 temperatures with oxides and with atmospheric oxidation almost instantaneously, whereby considerable of the aluminum added is ineffectually burned up.

To remedy these deficiencies, it has been suggested to use ferro-aluminum or a ferro-aluminum-silicon alloy. Such products have long been on the market but have not been utilized by the steel industry on account of 30 certain characteristic deficiencies of the products heretofore made. The ferro alloys thus produced contain appreciable quantities of carbon from approximately .50% to about 1.7%. This carbon content is present in these 35 alloys in the form of carbides, either a silicon

carbide, or aluminum carbide, or mixed carbides of silicon and aluminum, or of silicon, aluminum and iron. As is well known in the case of the ferro-silicon alloys, the presence of impurities such as carbides, tends to disintegrate such alloys, making them unfit for addition to molten steel. The presence of these carbides in the ferro-aluminum or ferro-aluminum-silicon alloys and their consequent disintegration is one of the reasons 55 that their commercial use in the steel industry has been prevented.

The improved composition of my present invention consists of an alloy with a minimum amount of carbon so as to be substantially carbide free and contains aluminum from 5% to 30%, preferably from 10% to 25%, and silicon from 60% to 90%, preferably between 60% and 75%; the remainder being principally iron, although usual impurities, or perhaps small quantities of other alloying metals, may be present. The carbon should be kept to a minimum not over .4% and preferably less than .15%. The alloy may be made by the addition of metallic aluminum into a bath of ferro silicon of the suitable composition in the ordinary electric furnace used for the manufacture of ferro silicon. The conditions under which a bath of molten ferro silicon exists in such a furnace are such as 70 to avoid contamination of the alloy produced by carbon.

Because of the relatively higher silicon content as compared with the aluminum content, a certain percentage of the silicon can be 85 retained in the steel with the retention of a much less quantity of aluminum than would be the case of an addition alloy having a lower silicon-to-aluminum ratio. This is of especial advantage in the manufacture of 90 steels which call for a relatively high percentage of silicon in the finished material.

This alloy, which is substantially free from carbides, can be obtained and kept in solid non-disintegrating lumps or masses suitable for addition to molten steel. This alloy has a specific gravity much greater than that of metallic aluminum and consequently enters into the body of the molten steel much more 95 readily. It does not react with the oxides and 100

other impurities present in the steel in such an instantaneous and violent manner as does metallic aluminum, but descends into the molten steel and interacts gradually, allowing the non-metallic impurities formed by the reaction to rise to the surface of the steel. Further, the product formed by the oxidation of the aluminum and silicon alloy together is an aluminum silicate, which has a very much lower melting point than aluminum, and therefore by the exothermic reaction between the ferro-silicon-aluminum and the molten steel, finds sufficient temperature to melt and rise to the surface through the body of the molten steel. Also, this alloy does not have the objectionable feature of introducing carbides into the steel, to thereby raise its carbon content, as would be the case with the carbide containing ferro-aluminum-silicon alloys heretofore used. This alloy further has the advantage that by its addition to steel its aluminum content acts more effectually on the body of steel, owing to its gradual and more positive action, not burning up quickly with the oxidation reaction as would be the case by the addition of metallic aluminum.

While I have described my alloy in its preferred composition, it is to be understood that the invention is not so limited but may be otherwise embodied within the scope of the following claims.

I claim:

1. A steel densifying and scavenging alloy, containing aluminum from 5% to 30%; silicon about 60% to 90%; the remainder being principally iron, and containing not over about .4% carbon.
2. A steel densifying and scavenging alloy, containing aluminum about 10% to 25%; silicon about 60% to 75%; the remainder being principally iron, and containing not over about .15% carbon.

In testimony whereof I have hereunto set my hand.

BYRAMJI D. SAKLATWALLA.

45

50

55

60

65